

Dec. 11, 1934.

J. U. DEVINE

1,983,934

METHOD AND APPARATUS FOR MAKING SEAMLESS TUBES

Filed July 18, 1931



INVENTOR

John U. Devine  
By Burns, Stubbins,  
Pardee & Blenko  
Attorneys.

## UNITED STATES PATENT OFFICE

1,983,934

METHOD AND APPARATUS FOR MAKING  
SEAMLESS TUBES

John U. Devine, Struthers, Ohio

Application July 18, 1931, Serial No. 551,597

9 Claims. (Cl. 80—62)

The present invention relates broadly to metal working as applicable to the manufacture of tubular objects, and more particularly to an improved method and apparatus for the manufacture of so-called seamless tubes.

In accordance with one method of manufacturing seamless tubes as now practiced, an ingot after being heated to the proper temperature is forged on a pilger mill, after which both ends are customarily cropped to a greater or lesser extent. In many cases also the pilgered ingot is sawed at intermediate points into two or more sections or lengths, depending upon the number of tubes which it is desired to produce from a given ingot. These lengths are then reheated in a reheating furnace, and after being brought to the proper temperature are taken to a plug mill effective for decreasing the wall thickness and smoothing the interior and exterior walls. To this end any desired number of passes is taken through the plug mill. The tubes thus formed are then taken to the reelers and sizing or reducing mills.

Inasmuch as a pilger mill necessarily operates to reduce the wall thickness of the pierced ingot, the surface of the ingot which is exposed, is materially greater when the ingot leaves the pilger mill than it is when the ingot leaves the piercing mill. Due to this greater surface, the reheating operation effects a very appreciable scaling, the amount of scale being comparatively large as compared to the weight of the metal being reheated. Thus from a standpoint of scale produced, it would be highly desirable to utilize a billet having thicker walls as it leaves the pilger mill. In accordance with the known manner of producing tubes, however, this would not be feasible, inasmuch as the plug mill would not be effective for reducing the wall thickness to the required extent.

Present methods of forming ingots also usually contemplate the utilization of an ingot of fairly large diameter as compared to the diameter of the finished tubes produced therefrom. Since the pilger mill usually operates in such manner that it produces an outwardly flared end on one end of the ingot, it is necessary in accordance with known processes of seamless tube manufacture wherein the pilger mill is utilized, to crop off the entire outwardly flared end portion, thus providing a length of substantially uniform outside diameter. The amount of cropping thus required averages in the neighborhood of 13%, this representing a large amount of waste as compared to the total weight of the pierced ingot.

The present invention has for one of its objects the utilization of an ingot of relatively smaller diameter, for a given sized tube, than has heretofore been used. In this manner the dimensions of the handling equipment may be correspond-

ingly reduced, which is of decided advantage particularly with respect to the reheating equipment.

Another object of the present invention is to provide a method such that the wall thickness of the intermediate article leaving the pilger mill is greater than that heretofore considered feasible, thus reducing to a corresponding extent the surface exposed to scaling during the reheating operation.

Still another object of the present invention is to afford a method by means of which scrap losses may be materially reduced.

In the accompanying drawing I have shown by way of illustration only, a preferred embodiment of the present invention. In the drawing:

Figure 1 is a diagrammatic plan view of a layout in accordance with the present invention;

Figure 2 is a perspective view partly broken away of a pierced billet or ingot;

Figure 3 is a longitudinal sectional view through a semi-finished article as produced in the pilger mill; and

Figure 4 is a view similar to Figure 3 of an article as produced in the second piercing mill.

Having reference more particularly to the diagrammatic showing of Figure 1 of the drawing, I have illustrated a layout comprising an ingot heating furnace 2 wherein the ingots or billets to be formed into tubes may be brought to the proper temperature. At this temperature the ingots are carried in any well known manner to a first piercing mill 3 wherein they are subjected to a piercing operation suitable for producing a hollow ingot or billet 4 substantially as illustrated in perspective in Figure 2 of the drawing. In this figure the pierced ingot or billet is shown as of substantially constant exterior diameter throughout the main body thereof, the exterior and interior walls 5 and 6 respectively at the ends extending in slightly converging relationship. In Figure 2 such a shape, which is characteristic of a piercing mill, is indicated in a much exaggerated scale.

After leaving the piercing mill the pierced ingots or billets may be delivered in any desired manner, as by a suitable conveyor 7, to a transfer track 8 cooperating at its ends with the rolls 9 of pilger mills driven in any customary or desired manner. Cooperating with the pilger mills are mandrel operating and feeding mechanisms 10.

In accordance with the present invention, it is contemplated that the pilger mills 9 will perform less forging than has heretofore been customary, thereby delivering an intermediate article 11, as illustrated in Figure 3, which will have a relatively thick wall, and thus a less surface available for scaling. This intermediate article has a substantially uniform outside dimension throughout the major portion of its length, but at the trailing 60

end has an outwardly flared portion 12, characteristic of the pilgering process. In view of the fact that this intermediate article has heretofore been passed directly to a plug mill, it has been necessary to crop the same so as to remove, entirely, the outwardly flared portion. To this end cropping has usually been effected along a line such as indicated at *a*—*a* in Figure 3. This cropping has been not only for the purpose of squaring up the intermediate article, but for the purpose of removing the portion of the ingot in which the segregation or piping usually appears, the ingot being presented so that such piping is contained within the thickened end portion 12. In accordance with my invention, the crop loss will be materially reduced by delivering the intermediate article from the pilger mills to hot saws 14 effective for sawing the same along a line such as indicated at *b*—*b* in Figure 3.

The sawed article with its fairly thick walls, will then be delivered to a conveying trough 15 and out to an inspection table 16. Here the billets may be inspected, and if found satisfactory, may be rolled into a reheating furnace 17. If, however, seams, scabs, or other defects show up at this point, the billets may either be chipped at the inspection table and made acceptable for further working, or may be conveyed out to a chipping or cross-over table 18 where they can be worked upon or conveyed either to a scrap pile or some other desired point, depending upon the disposition to be made thereof. In the reheating furnace the billets will be brought to the desired temperature for subsequent operations.

Inasmuch as the billet or ingot utilized in the first instance has a relatively smaller diameter than ingots or billets as heretofore utilized for the production of tubes of the same size, the dimensions of the reheating furnace may be smaller than the dimensions of reheating furnaces customarily provided. Furthermore, since the amount of forging effected by the pilger mill is less than that customarily resorted to, thus leaving a greater wall thickness, the billets leaving the pilger mill have a smaller overall length, thereby further contributing to the use of smaller reheating furnaces. This is advantageous not only from the standpoint of the cost of the installation, but also from the standpoint of compactness of the different units. The small amount of forging is desirable in that it not only gives a lighter load on the pilger mill with consequent less likelihood of roll breakage, but for the reason that it leaves a greater wall thickness effective for retaining a greater amount of the initial heat supplied in the furnace 2. This greater heat correspondingly reduces the heating period in the reheating furnace 17.

After a billet has been reheated in the reheating furnace 17, it is discharged therefrom onto a suitable conveying mechanism 19 by which it is delivered to a second piercing mill 20 which may be similar to the first piercing mill 3. This second piercing mill will produce an intermediate article 21 as illustrated in Figure 4, having end portions 22 as before described, and as characteristic of a piercing mill, with an intermediate portion of substantially constant diameter and cross section. The operation of the second piercing mill 20 will not only tend to decrease the wall thickness, but to increase the inner and outer diameters of the article and increase the length thereof. It will also be effective for dislodging any scale formed on either the inside or outside of the billet 25 during the reheating operation.

I am aware that it has heretofore been proposed to practice the so-called double piercing of an ingot in which the piercing occurred in successive steps. Such an operation as heretofore practiced, however, has not been satisfactory for the production of a billet for plug mill operation, due to the amount of working performed on the metal at the piercing mills, the amount of working being such that the ingot has been subjected to strains sufficiently severe to produce tearing thereof. In accordance with my invention, although successive piercing is utilized, the billets or ingots are subjected to an intermediate forging operation in the pilger mill, which operation is effective for refining the grain structure and increasing the strength of the metal, thus permitting a second piercing operation to be performed without danger of disruptive straining of the metal.

The piercing operation following the reheating is also desirable from the standpoint that it effects substantially complete removal of the scale formed by reheating. Heretofore when a billet has been passed directly from a reheating furnace to the plug mill, the scale has given considerable trouble. The scale being extremely hard, has a destructive action on such plugs. By the present invention, the scale is eliminated, thus reducing the wear on the plugs in the plug mill and giving the same a materially greater life.

In generally like manner, the less scale produced in the reheating furnace due both to the decreased heating time and the less surface area, is advantageously reflected in the second piercing mill.

The second piercing operation also enables the outwardly flared portion intermediate the lines *a*—*a* and *b*—*b* as shown in Figure 3 to be easily brought down to the desired thickness. A piercing mill being of much sturdier construction than a plug mill, and therefore capable of taking greater loads, makes possible the decrease in crop losses, since a piercing mill may readily compensate for the flaring left by the pilgering process. In addition to this, the piercing mill tends to produce tapered end portions, as before described. Heretofore it has been the practice to square saw the front ends of the billets coming from the pilger mills, and then feed the square sawed end over the plug in the plug mill. This often caused stoppages due to the act of trying to force the square edged, square-ended billet over the plug. This resulted in slipping at the plug mill, the slipping being augmented by the large amount of scale present.

The tapered ends characteristic of a piercing mill operation facilitate insertion of the article into the plug mill, and also eliminate any shock or jar on such mill at the time of insertion. The intermediate article may be given any number of passes in the plug mill, and the wall thickness reduced to substantially the finished thickness desired. Such plug mill is effective not only for removing irregularities produced in the article by the severe working in both the piercing mills and in the pilger mill and smoothing both the inside and outside surfaces, but also for giving to the articles the desired uniformity in wall thickness from end to end thereof.

By reference to Figure 1, it will be noted that the article upon leaving the second piercing mill 20 goes to a transfer table 23 effective for delivering the same to a plug mill 24 provided with the usual plug mill pusher 25. After the article has been subjected to the desired number of passes, it is discharged onto a suitable conveyor 26 from

which it may pass to reelers effective for rounding and increasing the diameter thereof, and thence to sizing machines constituting no essential part of the present invention.

- 5 For purposes of a clearer understanding of the present invention, and by way of illustration and not by way of limitation, it may be assumed that it is desired to produce a finished pipe having the outside diameter indicated in the first table below.
- 10 In such case I may advantageously utilize an ingot having a diameter as indicated in the second table:—

| 15 | Size of finished pipe (O.D.)                                                           | Ingot diameter                                                                           |
|----|----------------------------------------------------------------------------------------|------------------------------------------------------------------------------------------|
| 20 | 6 $\frac{1}{2}$<br>8 $\frac{1}{2}$<br>10 $\frac{1}{2}$<br>12 $\frac{1}{2}$<br>13<br>16 | 11 $\frac{1}{2}$<br>13 $\frac{1}{4}$<br>15<br>17 $\frac{1}{4}$<br>17 $\frac{1}{2}$<br>19 |

Assuming conditions as represented by the above tabulation, the first piercer, the pilger mill, the 25 second piercer and the plug mill may then be operated to dimension the article as indicated in the following tables:

| 30 | From first piercer<br>I.D.                                                                                        | From pilger mill                            |                                              | From second piercer        |                                                                                        | From high mill             |                                                                                        |
|----|-------------------------------------------------------------------------------------------------------------------|---------------------------------------------|----------------------------------------------|----------------------------|----------------------------------------------------------------------------------------|----------------------------|----------------------------------------------------------------------------------------|
|    |                                                                                                                   | I.D.                                        | O.D.                                         | I.D.                       | O.D.                                                                                   | I.D.                       | O.D.                                                                                   |
| 35 | 4 $\frac{1}{2}$<br>6 $\frac{1}{2}$<br>8 $\frac{1}{2}$<br>10 $\frac{1}{2}$<br>10 $\frac{1}{2}$<br>13 $\frac{1}{2}$ | 3 $\frac{1}{4}$<br>6<br>8<br>10<br>10<br>13 | 5 $\frac{1}{4}$<br>8<br>10<br>12<br>12<br>15 | x<br>x<br>x<br>x<br>x<br>x | 7<br>9 $\frac{1}{4}$<br>11 $\frac{1}{4}$<br>13 $\frac{1}{2}$<br>13 $\frac{1}{4}$<br>17 | y<br>y<br>y<br>y<br>y<br>y | 6 $\frac{1}{2}$<br>8 $\frac{1}{2}$<br>10 $\frac{1}{2}$<br>12 $\frac{1}{2}$<br>13<br>16 |

40 The values *x* indicated in the above table will depend on the wall thickness desired in the finished pipe, while the values *y* depend also upon the thickness desired in the wall of the finished pipe, these being subject to change as required to meet specified conditions.

45 In accordance with the present invention, it will be apparent that I provide a process characterized by double piercing with a refining operation intermediate the same, the refining being effective for increasing the strength and improving the 50 grain structure of the article. This constitutes one of the advantages of the present invention.

A further advantage of the invention arises 55 from the fact that a double piercing operation is utilized, thus decreasing the load on each piercing mill, and making it possible to employ successive piercing operations without danger of rupturing the metal or subjecting the same to objectionable strains.

60 Still another advantage of the present invention arises from the fact that by reducing the wall thickness in the first piercing mill, the area of the intermediate article delivered by the pilger mill for reheating purposes may be kept at a minimum, thus conserving heating time and reducing scale formation.

65 Further advantages arise from the use of a relatively smaller diameter ingot for the production of a given sized pipe or tube and from the consequent possibility of reducing the size of the 70 reheating furnace.

Another advantage of the invention is inherent in the reduction in crop losses made possible by

pilgering an article intermediate successive piercing steps, and from the improved operation of a plug mill occasioned by piercing an article after a pilgering step.

Other advantages will be apparent from the foregoing description taken in connection with the accompanying drawing forming a part thereof.

While I have herein illustrated and described a preferred method and apparatus for carrying out the present invention, it will be understood that changes in the steps employed as well as in the apparatus utilized for performing the same, may be made without departing either from the spirit of my invention or the scope of my broader 15 claims.

I claim:

1. In the method of forming seamless tubes, the steps comprising subjecting the product of a pilger mill to a piercing operation and then 20 rolling the same in a plug mill.

2. In the method of forming seamless tubes, the steps comprising piercing an ingot, pilgering the pierced ingot, piercing the product of the pilger mill, and thereafter rolling such product 25 in a plug mill.

3. In the method of forming seamless tubes, the steps comprising heating an ingot, piercing and pilgering the same, reheating the product of the pilgering process, subjecting the pilgered 30 product to a piercing operation, and then smoothing and sizing the same by subjecting the same successively to plug mill, reeling and sizing operations.

4. In the method of forming seamless tubes, 35 the steps comprising subjecting a pierced ingot to a pilgering process, tapering the end portions of the pilgered article, and delivering the same to a plug mill.

5. In the method of forming seamless tubes, 40 the steps comprising subjecting a pierced ingot to a pilgering process, tapering the end portions of the pilgered article by subjecting the same to a piercing operation, and delivering the same to a plug mill.

6. In the method of forming seamless tubes, 45 the steps comprising piercing an ingot, pilgering the same, cropping the pilgered article so as to retain a portion of the flared end, and thereafter removing the flared portion by subjecting the same to a piercing operation.

7. In a tube making system, means for piercing ingots, means for reducing the wall thickness of the pierced ingots to produce semi-finished tubes, means for again piercing the semi-finished tubes, means for then heating the tubes and a plug mill for changing the diameter of the tubes received from the second piercing means and heating means.

8. In the method of preparing articles for operation in a plug mill, the steps comprising subjecting the same to a plurality of piercing operations with an intermediate pilgering operation, and then rolling such product in a plug mill.

9. In the method of preparing articles for operation in a plug mill, the steps comprising subjecting the same to a plurality of piercing operations with an intermediate forging operation, and then rolling the product in a plug mill.

JOHN U. DEVINE.